# EUROPEAN PATENT SPECIFICATION

(11) **EP 1 163 315 B1**
(45) Date of publication and mention of the grant of the patent: **16.04.2008**
(21) Application number: 00907813.0
(22) Date of filing: 06.03.2000
(51) Int. Cl.: C10L 1/32

(54) **COMPOSITIONS FOR PREPARING WATER-IN-OIL MICROEMULSIONS**
ZUSAMMENSETZUNGEN FÜR DIE HERSTELLUNG VON WASSER IN ÖL MIKROEMULSIONEN
COMPOSITIONS DESTINEES A LA PREPARATION DE MICROEMULSIONS EAU-DANS-HUILE

(30) Priority: 06.03.1999 GB 9905099; 17.07.1999 GB 9916754
(43) Date of publication of application: 19.12.2001
(73) Proprietor: PALOX offshore S.A.L., Beit-Mery (LB)
(72) Inventor: ABU-JAWDEH, Pauline, London SW1X 9PD (GB); MARTIN, David, Netherton, Liverpool L30 6YF (GB)
(74) Representative: Buckley, Guy Julian
(86) International application number: PCT/GB2000/000800
(87) International publication number: WO 2000/053699

(56) References cited:
- WO-A-98/50139
- FR-A- 2 373 328
- US-A- 3 346 494
- US-A- 3 876 391
- US-A- 4 770 670

## Description

The present invention relates to a water-in-fuel emulsion, wherein the average droplet size of the water phase in the emulsion is no greater than 0.1 µm, and uses thereof.

Lubricants used in the production of metals etc. are known to be flowable systems which can be assigned to one of the following three categories.
Neat oils: are as the name suggests base oil that incorporates specialist additives to overcome wear, foaming etc. These lubricants are the most lubricious giving good surface finishes to produced pieces. However, they are also the poorest at cooling the tool/metal interface. This means that the machining rate is much reduced in comparison to soluble oils. Overall neat oils have little in the way of disadvantages other than a lack of coolancy, as they are easy to handle, have a long sump life, can be reconditioned, and are easy to filter and dispose of as and when necessary.
Soluble oils: consist of a concentrate, which is diluted with water by up to 50 times. As they are predominantly water they have a very high degree of coolancy. However, this is at the expense of lubricity and though the metal can be worked very quickly the surface finish is generally poor. Due to their high water content the possibility of both corrosion and bacterial growth arises requiring additional additives such as corrosion inhibitors and biocides. The latter being liable to cause dermatitis thus making handling more of a problem. Disposal of these oils is also very difficult since they cannot be easily incinerated. They are generally demulsified, which is a very expensive procedure.
Water-in-oil emulsions: have been used to give a lubricant that has properties somewhere between the neat and soluble oils. However, these oils are usually unstable and have many of the same problems as the soluble oils. Attempts have been made previously to formulate stable invert emulsions e.g. WO 92/07053, however, these emulsions although having a much reduced droplet size are inherently unstable. This leads to separation problems and also both corrosion and bacterial growth.
Fuels: are defined as hydrocarbon feedstock for powering an engine or other such machinery. The invention uses all fuel types i.e. diesel, kerosene, petrol (leaded or unleaded) and mixtures thereof

The use of fuel emulsions has been undertaken previously by many applicants. However, the emulsions formed are of a large water droplet size giving a milky appearance. These emulsions require a number of secondary additives such as corrosion inhibitors and bactericides to overcome addition of the water phase. These emulsions due to their large water droplet size also exhibit instability that leads to fuel/water separation. Naturally, this is unwelcome as it may lead to problems with not only machine failure but also problems with loss of production in say a diesel-powered generator.

The present invention describes a composition that allows that formation of translucent microemulsions having a water droplet size of less than 0.1 µm and preferably less than 0.01 µm. This small droplet size not only gives an appearance with is more aesthetically pleasing to the user but offers several major advantages over the present systems. The translucency imparted due to the small droplet size negates the need for both corrosion inhibitors and bactericides. An improvement in the lubricity of the emulsions is also gained probably due to the surfactants, which help to stabilise the emulsion. These systems are also thermodynamically stable by nature and will therefore not have the inherent instability of typical systems.

The advantages seen in these systems will not deter from the advantages of using water-in-fuel emulsions i.e. cleaner emissions, reduced particulate matter and improved combustion rates (leading to better fuel consumption). WO 98/50139 describes the use of microemulsions in several industrial lubricant applications including cutting oils, hydraulic fluids, gear oils and grinding fluids. The composition for preparing the microemulsion comprises i) a fatty acid amine ethoxylate ii) C6-C15 alcohol ethoxylate; and optionally iii) tall oil fatty acid amine.

US-A-3 876 391 discloses a process for preparing water-in-petroleum type of micro emulsions.

The present invention addresses problems of the prior art. Aspects of the present invention are defined in the appended claims.

The present invention provides new water-in-fuel emulsions wherein the fuel may be as defined below. The droplets of the water phase of the emulsion have an average droplet size of no greater than 0.1 µm. These emulsions are clear translucent emulsions. Any reference in the present specification to "a water-in-fuel emulsion, wherein the average droplet size of the water phase of the water-in-fuel emulsion is no greater than 0. 1 µm ", is analogous to the term "a water-in-fuel emulsion wherein the emulsion is a clear translucent emulsion".

The present invention provides a stable emulsion. The emulsion is of a continuous fuel phase in which water droplets, having an average droplet size of no greater than <0.1 µm are dispersed. The resultant clear translucent emulsion is thermodynamically stable and offers both high lubricity and cooling properties.

Thus, a first aspect of the invention relates to a water-in-fuel emulsion, wherein the average droplet size of the water phase of the water-in-oil emulsion is no greater than 0.1 µm.

The present invention provides a water-in-fuel emulsion that, due to the extremely small droplet size, cannot support microbial growth.

The mixture ratios of the fuel and water phases of the emulsion can be varied depending on the application of the emulsion. Generally speaking, the fuel comprises at least about 80% by weight, based on the total of the fluid phases, fuel and water. Generally speaking, the fuel phase comprises no greater than about 90% by weight or about 95% by weight. (Each percentage by weight is based on the total of the fluid phases fuel and water).

The emulsifier composition is preferably chosen to minimise the amount of emulsifier to form a microemulsion for a given base fluid. Typically, the composition comprises between 5 and 30% by weight of emulsifier. Preferably, between 5 and 20% and more preferably between 5 and 10%.

In general, the water-in-fuel emulsions comprise a C₆-C₁₅ alcohol ethoxylate, an amine ethoxylate and a polyisobutylsuccinimide or sorbitan ester.

The fuel in the present invention is selected from diesel, kerosine, petrol (leaded or unleaded) and mixtures thereof.

In a further preferred aspect the present invention may provide an emulsion comprising (i) 10 parts water; (ii) 90 parts diesel fuel; and (iii) emulsifying agents as defined herein, in amount of 14 parts by volume relative to the total fuel and water.

In a further preferred aspect the present invention may provide an emulsion comprising (i) 10 parts water; (ii) 90 parts unleaded petrol; and (iii) emulsifying agents as defined herein, in amount of 10 parts by volume relative to the total fuel and water.

In a further preferred aspect the present invention may provide an emulsion comprising (i) 10 parts water; (ii) 90 parts diesel fuel; and (iii) emulsifying agents as defined herein, in amount of 12 parts by volume relative to the total fuel and water.

An important area of use for the new water-in-fuel emulsions of the present invention is in the heavy duty diesel engine market, particularly trucks, buses and other heavy duty transport vehicles, although the present invention is not limited to this application area.

The water phase used can be taken directly from the local water supply.

The emulsion may comprise additional components. These additional components may be incorporated to improve anti-wear or extreme pressure properties or act as an antifreeze, for example, ethylene glycol. The requirement to add additional components may be dictated by the application area in which the invention is used. Suitable additional components, and the requirement therefor depending on application area, will be apparent to those skilled in the art.

## Claims

1. A water-in-fuel emulsion, wherein the average droplet size of the water phase of said emulsion is no greater than 0.1 µm, comprising
(a) water;
(b) a fuel selected from diesel, kerosene, petrol (leaded or unleaded), and mixtures thereof; and
(c) emulsifying agents comprising i) a C₆-C₁₅ alcohol ethoxylate, ii) polyisobutylsuccinimde or a sorbitan ester, and iii) an amine ethoxylate.

2. A water-in-fuel emulsion as claimed in any one of claim 1, wherein said emulsion comprises:
(a) 10 parts water;
(b) 90 parts diesel fuel; and
(c) 14 parts by volume relative to the total fuel and water of said emulsifying agents.

3. A water-in-fuel emulsion as claimed in any one of claim 1, wherein said emulsion comprises:
(a) 10 parts water;
(b) 90 parts diesel fuel; and
(c) 12 parts by volume relative to the total fuel and water of said emulsifying agents.

4. A water-in-fuel emulsion as claimed in any one of claim 1 wherein said emulsion comprises:
(a) 10 parts water;
(b) 90 parts unleaded petrol; and
(c) 10 parts by volume relative to the total fuel and water of said emulsifying agents.

5. A water-in-fuel emulsion as claimed in claim 1, wherein the fuel comprises at least 80 % by weight, based on the total weight of the water and fuel.

6. A water-in-fuel emulsion as claimed in claim 1, wherein the fuel comprises no more than 90 % by weight, based on the total weight of the water and fuel..

7. Use of a water-in-fuel emulsion as claimed in any one of claims 1-6 as a fuel oil.

8. Use in the heavy engine diesel market of a water-in-fuel emulsion as claimed in any one of claims 1-6.

## Patentansprüche

1. Eine Wasser-in-Kraftstoff-Emulsion, wobei die durchschnittliche Tröpfchengröße der Wasserphase dieser Emulsion nicht größer als 0,1 µm ist und die Emulsion Folgendes umfasst:
(a) Wasser;
(b) einen Kraftstoff ausgewählt aus Diesel, Kerosin, Benzin (verbleit oder bleifrei), und Mischungen derselben; und
(c) Emulgatoren umfassend i) ein C₆ - C₁₅ Alkoholethoxylat, ii) Polyisobutylsuccinimid oder ein Sorbitanester und iii) ein Aminethoxylat.

2. Eine Wasser-in-Kraftstoff-Emulsion wie in Anspruch 1 beansprucht, wobei die Emulsion Folgendes umfasst:
(a) 10 Teile Wasser
(b) 90 Teile Dieselkraftstoff; und
(c) 14 Volumenanteile Emulgatoren mit Bezug auf die Gesamtmenge an Kraftstoff und Wasser

3. Eine Wasser-in-Kraftstoff-Emulsion wie in Anspruch 1 beansprucht, wobei die Emulsion Folgendes umfasst:
(a) 10 Teile Wasser;
(b) 90 Teile Dieselkraftstoff; und
(c) 12 Volumenanteile Emulgatoren mit Bezug auf die Gesamtmenge an Kraftstoff und Wasser

4. Eine-Wasser-in-Krafstoff-Emulsion wie in Anspruch 1 beansprucht, wobei die Emulsion Folgendes umfasst:
(a) 10 Teile Wasser
(b) 90 Teile Dieselkraftstoff; und
(c) 10 Volumenanteile Emulgatoren mit Bezug auf die Gesamtmenge an Kraftstoff und Wasser.

5. Eine Wasser-in-Kraftstoff-Emulsion wie in Anspruch 1 beansprucht, wobei der Kraftstoff mindestens 80 Gew. % mit Bezug auf das Gesamtgewicht des Wassers und Kraftstoffs ausmacht.

6. Eine Wasser-in-Krafstoff-Emulsion wie in Anspruch 1 beansprucht, wobei der Kraftstoff nicht mehr als 90 Gew. % mit Bezug auf das Gesamtgewicht des Wassers und Kraftstoffs ausmacht.

7. Verwendung einer Wasser-in-Krafstoff-Emulsion wie in einem der Ansprüche 1 - 6 beansprucht als Schweröl.

8. Verwendung einer Wasser-in-Kraftstoff-Emulsion wie in einem der Ansprüche 1 - 6 beansprucht im Bereich leistungsstarker Dieselmotoren.

## Revendications

1. Emulsion d'eau dans du carburant, dans laquelle la taille moyenne des gouttelettes de la phase aqueuse de ladite émulsion ne dépasse pas 0,1 µm, comprenant :
(a) De l'eau;
(b) Un carburant sélectionné entre le diesel, le kérosène (avec ou sans plomb), et un mélange de ceux-ci ; et
(c) Des agents émulsifiants comprenant : i) de l'éthoxylate d'alcool C₆-C₁₅, ii) du polyisobutylsuccinimide ou un ester de sorbitan, et iii) un éthoxylate amine.

2. Emulsion d'eau dans du carburant, comme revendiquée dans la revendication 1, dans laquelle ladite émulsion comprend :
(a) 10 parties d'eau ;
(b) 90 parties de carburant diesel: et
(c) 14 parties par volume par rapport à l'ensemble du carburant et de l'eau, desdits agents émulsifiantes.

3. Emulsion d'eau dans du carburant, comme revendiquée dans la revendication 1, dans laquelle ladite émulsion comprend :
(a), 10 parties d'eau;
(b) 90 parties de carburant diesel ; et
(c) 12 parties par volume par rapport à l'ensemble du carburant et de l'eau, desdits agents émulsifiants.

4. Emulsion d'eau dans du carburant, comme revendiquée dans la revendication 1, dans laquelle ladite émulsion comprend :
(d) 10 parties d'eau;
(e) 90 parties de carburant diesel, et
(f) 10 parties par volume par rapport à l'ensemble du carburant et de l'eau, desdits agents émulsifiants.

5. Emulsion d'eau dans du carburant, comme revendiquée dans la revendication 1, dans laquelle le carburant comprend au moins 80% en poids, en se basant sur le poids total de l'eau et du carburant.

6. Emulsion d'eau dans du carburant, comme revendiquée dans la revendication 1, dans laquelle le carburant comprend au moins 90% en poids, en se basant sur le poids total de l'eau et du carburant.

7. Utilisation d'une émulsion d'eau dans du carburant, comme revendiquée dans l'une quelconque des revendications 1 à 6, comme du combustible.

8. Utilisation sur le marché des moteurs diesel lourds d'une émulsion d'eau dans du carburant, comme revendiquée dans l'une quelconque des revendications 1 à 6.
